

Patented Dec. 6, 1927.

1,651,665

## UNITED STATES PATENT OFFICE.

LINN BRADLEY, OF MONTCLAIR, NEW JERSEY, AND EDWARD P. MCKEEFE, OF NEW YORK, N. Y.

### MANUFACTURE OF PULP AND PAPER.

No Drawing.

Application filed February 8, 1922. Serial No. 535,034.

This invention relates to improvements in the commercial manufacture of pulp and paper from wood, and includes improvements in the production of the pulp and paper, as well as in the pulp and paper themselves. The invention also includes a regenerative process of pulp manufacture in which the residual liquors are treated for the regeneration of cooking liquors for use in the further carrying out of the process.

In the ordinary soda process so-called of manufacturing pulp from wood, the wood chips are cooked with a cooking liquor consisting essentially of caustic soda. In order to complete the cooking operation, the amount of the caustic soda required is such that a considerable part of the wood fibres are injured or destroyed or over-cooked, with a corresponding decrease in yield and quality of pulp produced. If the soda process is carried out with an amount of caustic soda which does not materially injure the fibres, the operation is unreliable or incomplete and the product is unsatisfactory. If, for any reason, the cooking operation is run overtime, as, for example, where a breakdown has occurred in some part of the pulp mill, or in case of delay or an accumulation of pulp in some part of the mill, such that a digester cannot be discharged until the accumulated pulp has been worked off, the overcooking of the digester charge, with the usual soda cooking liquors, may result in overcooking, and injury or destruction such that the pulp is of decreased value and reduced yield and may even be difficult to handle. The overcooking of the pulp may cause a partial gelatinization of the fibres or may make the pulp more mushy and more difficult to wash and dry and handle in its subsequent manipulation in the pulp mill. Overcooking, in the case of ordinary soda cooking liquors, may not only give difficulty in the treatment of the pulp, but may likewise give difficulty in the treatment of the residual liquors, which contain an increased amount of dissolved fibres.

The pulp produced by the soda process, for example, from poplar (aspen) wood, is yellowish or brownish in tint, and, the bleached pulp on heating, generally turns yellowish. The pulp is often of a mushy character, which is difficult to handle satisfactorily in the pulp mill. The pulp made

by the soda process, for example, from poplar (aspen) wood, has been of such inferior properties that it has been considered and used as a short fibre filler in admixture with long fibre pulp which gives strength to the resulting paper. For example, in the manufacture of paper, it has been customary to use from about 50 to 70% of long fibre sulphite pulp (e. g. produced from spruce wood) in admixture with from 50 to 30% of soda pulp made from poplar wood, depending upon the weight and strength of the paper (e. g. book and magazine paper) to be manufactured. In order to produce such a composite paper it has been customary for a soda pulp and paper mill either to buy sulphite pulp to admix with the short fibre soda pulp, or to operate both the soda and the sulphite processes independently to produce the respective soda and sulphite pulps, so that the long fibre sulphite pulp could be mixed with the short fibre soda pulp, the soda pulp being considered merely a filler, and the sulphite pulp being relied upon to give strength.

When long fibre sulphite pulp is thus admixed with soda pulp, it is customary to subject the mixed fibres to a beating operation in order to convert the sulphite fibres into the proper condition. This beating operation may overbeat the softer soda pulp fibres, particularly with a pulp of mushy character which has insufficient strength to withstand the beating operation, and this overbeating may further injure the fibres and cause them to fill the voids of the pulp and paper in such a way as to injure the felting properties or the subsequent handling of the pulp and paper.

Owing to the delicacy of the ordinary soda process, it is difficult, even in a well-regulated mill, to keep all parts of the pulp-making process in balance, so that the successive parts of the process can operate in sequence and on a regular schedule, and difficulties frequently arise on account of imperfect operating conditions. For example, in the case of a pulp which is difficult to drain or to bleach, the slowing up of the drainers or bleachers may hold up the digesters a longer time than required for the completion of the cooking operation, thus preventing the blowing off of the digesters until the part of the mill ready to receive

the charge has been freed from the previous charges, with resulting overcooking of the pulp and injury thereto.

According to the present invention, the difficulties and disadvantages of the ordinary soda process are largely overcome or minimized and the cooking of the wood in the digesters is carried out in a new and improved way which gives a superior pulp and paper, which enables the residual liquors to be treated in a more advantageous way, and which enables the mill to be more readily balanced and to be operated in a more reliable way. The nature and advantages of the invention will more fully appear from the following more detailed description of the invention.

According to the present invention, the cooking operation is carried out with a cooking liquor consisting essentially of caustic soda together with normal sodium sulphite, with the caustic soda present in preponderating amount, that is, with the amount of sodium present as sulphite not exceeding the amount of sodium present as caustic soda, and ordinarily with the amount of sodium sulphite smaller in sodium content than that of the caustic soda, for example, from 10 to 25% of the total sodium present or somewhat more. The caustic soda, although in preponderating amount, is nevertheless so controlled in amount and concentration in the cooking liquor that it does not exert any excessively destructive action on the fibres of the wood.

We have found that by cooking wood, for example, poplar wood, with such a composite cooking liquor, the objectionable injury to the pulp resulting from the ordinary soda process is largely avoided, and a new and superior pulp can be produced with fibres of sufficient strength and of improved properties such that they can be used alone, without admixture of long fibre sulphite pulp, in the manufacture of paper.

We have found further that the residual liquors are themselves of distinctive composition and can be readily treated for the regeneration of the cooking liquors, even by the ordinary procedure and apparatus employed in the treatment of black liquors from the soda process, (provided the operations are specially regulated) and even though the residual liquors and cooking liquors of the present invention contain a considerable amount of sulphite.

The process of the present invention is of more or less general application. It is of particular value for the treatment of poplar wood, and, by its use, a new and improved pulp can be produced from poplar wood with fibres having such improved physical and chemical properties that the pulp can be more readily handled in the mill, is freer flowing and freer working throughout the

mill than the ordinary soda pulp, drains more freely, washes quicker, bleaches more easily, is freer from objectionable properties such as mushiness or a hydrated or gelatinous character, and, as above stated, gives a paper of superior strength and properties even without admixture of long fibre sulphite pulp.

The process is also applicable to other woods than poplar, for example, to hard woods or deciduous woods such as birch, beech and maple, as well as coniferous woods such as spruce, pines (e. g. Norway or Loblolly) etc. Even dense woods, such as certain of the hard woods, can be readily treated and a new and improved pulp produced therefrom, with fibres having characteristic and distinctive physical and chemical properties.

In carrying out the process, the wood may be prepared in the customary way, by barking, clipping and crushing and by screening to take out dirt, with the chips made of more or less uniform size by the chipping and crushing operation. The chips suitably prepared may be charged into the digesters in much the usual way, for example, by first introducing part of the chips, then introducing the chips and liquor simultaneously while keeping the chip level above the liquor level, and turning on steam to heat the liquor, drive out air, and compact the chips.

The cooking liquor, as above stated, is a composite liquor consisting essentially of caustic soda and normal sodium sulphite so that the cooking liquor combines the reagents of the caustic soda process and of the sulphite process, although the liquor is not acid (as is the liquor in the acid sulphite process) nor is it as strongly alkaline as the liquor of the ordinary soda process. By reducing the amount of caustic soda and substituting normal sodium sulphite therefor, we have found that the objections and difficulties of the ordinary soda process are very largely overcome. The cooking liquor may, for example, for poplar wood, have a strength of about 15 or 16 Twaddell and may be e. g. of 90% causticity based on  $Na_2CO_3$ . In general, the liquors may contain from 50 to 60 grams per liter of caustic soda and from 10 to 25 grams per liter of normal sodium sulphite, although an even larger amount of sulphite, up to an amount equal to that of the caustic soda may be used. With dense hard wood a radically increased amount of the reagents should be used and it is one advantage of the invention that such increased amounts can be used as hereinafter set forth.

The cooking liquor in the first instance may be made in any suitable way, for example, by adding sulphur dioxide to a suitable solution of caustic soda or to a suitable solution of sodium carbonate before caustici-

zation. The composite cooking liquor may also be made, in a simple and advantageous way, from the ordinary soda and sulphite liquors used respectively in the soda and acid sulphite processes. Where acid calcium sulphite liquors are available they may be made to react with alkaline liquors, with precipitation of neutral calcium sulphite which may be returned to the absorption towers of the sulphite process or otherwise utilized, e. g. with sodium acid sulphate to form sodium sulfite and calcium sulfate or gypsum.

In continued operations, it is only necessary to provide a sufficient amount of the reagents to make up for losses in the process, inasmuch as the cooking liquors can be readily regenerated from the residual liquors, in a manner hereafter more fully described.

The following specific example will further illustrate the invention as applied to poplar wood: Three and three-fourths cords of wood chips, (i. e. 3 $\frac{3}{4}$  cords measured before chipping) made up of about 90% poplar wood and 10% bass wood were charged into the digester together with about 460 cubic feet of cooking liquor containing 1515 pounds of caustic soda, and 488 pounds of sodium sulphite, together with small and incidental amounts of sodium carbonate (resulting from incomplete causticizing) and of sodium sulphide (incidentally produced in the regenerating operation). Small amounts of sodium sulfide, incidentally produced during the regenerative process, are advantageously present in the cooking liquor, giving a composite cooking liquor containing caustic soda in preponderating amount, together with sodium sulfite and sodium sulfide. The digester was about 7 feet inside diameter and about 25 feet in height over all. The digester was heated by the direct introduction of steam into the bottom of the digester. About two hours was required to bring the digester to pressure and the charge was cooked for a period of four hours under a steam pressure of 110 to 120 pounds, some of the air and steam at the top of the digester being relieved from time to time to promote the circulation and distribution of heat in the digester. The charge was then blown from the digester to the blow pit, then conveyed to a storage tank with a perforated false bottom where the liquor was drawn off and the pulp washed by displacement, the residual liquor and the concentrated wash water being conveyed to a storage tank for concentrated liquor, and the dilute wash water being separately stored and used to wash out the blow pit.

The above example is typical for poplar wood, but the specific conditions of this example are capable of variation. For example, instead of circulating the liquor by a steam jet at the bottom of the digester, cir-

culation can be effected by means of a pump.

In the cooking operation, a considerably less amount of the wood goes into solution than in the ordinary soda process. This results in an improvement both in the amount and properties of the pulp and in the composition and treatment of the residual liquors. Because of the increased amount of pulp produced, the storage tanks and apparatus employed in the subsequent treatment of the pulp may require to be somewhat increased in their capacity as compared with apparatus employed in treating ordinary soda pulp. Lower yields of pulp generally will be produced with older woods than with green sound wood. The wood may vary somewhat in its water content, and due allowance should be made for this in carrying out the process. Ordinary poplar wood used by us contained about 15 to 20% of water, and the above example refers to wood of such a water content. Where the wood has been in the water for a considerable time, its moisture content may be as high as 50% or higher.

One of the important advantages of the cooking process of the present invention is that moderate overcooking of the charge in the digester does not injure the pulp to any objectionable extent, so that overcooking is much less objectionable than in the ordinary soda process.

Another important and characteristic advantage of the invention is that a considerably increased yield of pulp can be produced from the wood than is produced in the ordinary soda process. In the case of poplar wood, for example, this increase may amount to 10% or more, while the pulp itself will be of greatly improved properties which distinguish it from ordinary soda pulp. Where, for example, a yield of about 1050-1100 pounds of air dry pulp is obtained from a cord of poplar wood according to the ordinary soda process, a yield of around 1200 or 1300 pounds or more of pulp (air dry) can be readily produced according to the improved process of the present invention; while the pulp will also be a superior pulp which can be more readily handled and which can be used for purposes and with advantages which distinguish it from ordinary soda pulp. The pulp is more uniform and is freer running through the mill. The pulp is characterized by increased fibre strength, freedom from objectionable mushiness, and contains fibres having physical and chemical properties and characteristics which distinguish it from the ordinary soda pulp produced from the same wood.

In its subsequent treatment by draining, washing, screening, thickening, bleaching, etc., the pulp is freer than ordinary soda pulp and can be more readily handled and with less difficulty. The pulp can be bleached and

the bleached pulp has superior properties. The spent bleach-liquor can be removed in any suitable way and the bleached pulp can then be converted into sheets and dried or 5 conveyed to the paper mill and used for the manufacture of a superior paper. For the manufacture of unbleached pulp or paper, the bleaching can be omitted. When the pulp is being subjected to beating, the beaters can be operated with considerably less power than when the usual mixtures of ordinary soda pulp and sulphite pulp are treated. The new pulp can also be more readily freed from water when subjected 10 to squeezing between rolls in the manufacture of pulp or paper sheets therefrom. In the drying of the pulp, or paper made therefrom, less heating is required than in the case of ordinary soda pulp. The water appears to be held in the pulp in a different 15 way from that in which it is held in ordinary soda pulp. In particular, the water seems to be held in such a way that it comes away from the fibres more readily, perhaps due to the fact that the fibres are not gelatinized or hydrated to such an extent and do not contain so much water intimately combined therewith, as in the case of ordinary 20 soda pulp.

30 The advantages of the new pulp are particularly marked when the pulp is used for the manufacture of paper. The pulp (bleached or unbleached), after screening, thickening and beating, and after the addition 35 of chemicals or fillers (e. g. alum, sizing, coloring material, fillers, etc.,) can be run through the refining engine or Jordan engine and then to the paper machine. For the heavier weights of paper, it is possible 40 to make excellent book or magazine paper entirely of poplar pulp, without admixture of long fibre sulphite stock. Owing to the absence of admixed sulphite fibres, the stock does not require as much beating as is required by the ordinary admixtures of sulphite and soda pulps, a light brushing in 45 the beaters usually being sufficient. After the refining operation the pulp can be run through the stock chest and then onto the 50 paper machine in regulated amount to give paper of the desired weight. The paper sheet can be formed in much the usual way, but the sheet dries easier and with less shrinkage than ordinary mixed soda and 55 sulphite paper. For example, where previously it was necessary to use a steam pressure of 18 pounds on the drying rolls of the paper machine, it was found sufficient to use one and one-half pounds of steam pressure 60 on the same dryer in drying the improved paper of the present invention (made for example from poplar wood). The water can more readily be squeezed out of the sheet on the squeeze rolls, and the remaining 65 water can more readily be removed on the

heated drying rolls. The new paper can also be formed more rapidly, owing to the increased speed at which it can be dried. In one instance, in the case of a 97 pound paper, the paper was dried at the rate of 70 about 115 feet per minute or about 40 feet faster than paper made from admixed soda pulp of ordinary grade and sulphite pulp. The paper also shrinks less in drying on the paper machine, thus making it possible to 75 cut sheets of increased width from the paper. The paper is also more uniformly formed and is strong enough to stand additional pressure if necessary at the calender rolls, so that it can be given a softer finish and a 80 higher finish if desired.

The improved paper of the present invention made, for example, from poplar wood, is of particular value for use as book paper, where a soft pliable, durable paper is desired which will lay flat and which will print without fuzzing or the raising of the fibre. It has a characteristic sheen or velvety finish and a surface which readily takes a finish 85 and which can be erased without raising the 90 fibre. It has a characteristic brightness or brilliancy of color. Owing to the more uniform character of the sheet, and the fact that it does not shrink as much in drying, the sheet is much safer on the paper machine 95 and there is less danger of breakage and interference with continuous operation.

The advantages of the new paper are illustrated by a comparison of it with ordinary book paper made from admixed soda pulp (poplar) and sulphite pulp (spruce). Heretofore in order to make paper of sufficient strength, at least about 30% of long fibre sulphite pulp was required in the case of the heavier weights of paper, such as 70 pound 100 stock, while 70% of sulphite pulp was commonly used in lighter paper, such as 40 pound stock. With the new pulp, however, it has been found possible to omit entirely 105 the admixture of long fibre sulphite pulp 110 for making the heavier weights of paper. For example, a 70 pound paper made entirely of the new pulp (from poplar wood) was found, when tested in a Mullen tester, to have a breaking strength of 27 pounds 115 as compared with a breaking strength of 24 pounds for a paper of the same weight made from admixed soda and sulphite pulp according to methods heretofore commonly used. (In referring to a 70 pound paper 120 we mean that a ream of 500 sheets of the paper of a standard size of 25" x 38" weighs 70 pounds.)

The paper, when made entirely of pulp, produced according to the present invention, 125 for example, from poplar wood, will be of a substantially uniform character in the sense that it will be made up entirely of fibres of substantially uniform length and properties, as distinguished from paper made up of 130

fibres that have been broken down by over-cooking (e. g. by the ordinary soda process) or by overbeating of the soft fibres of the soda process, due to the beating of the admixed long fibre sulphite pulp in admixture with the short fibre soda pulp. One important characteristic of the new pulp and of the paper made therefrom is that a minimum of beating is required to convert the pulp into a suitable form for paper making so that the fibres of the paper are not injured to an objectionable degree by the beating operation, while they are of such an improved character, in composition and properties, that they undergo such beating as is necessary without any material breaking down of the fibres, so that the fibres in the finished paper are essentially those of the original wood, as modified by the cooking and bleaching operation which separates the non-fibrous constituents, and by the mild beating operation which completes the treatment of the fibres for paper making purposes. In so far as we are aware, we are the first to produce an improved paper of this character, made up entirely of what is commonly considered short fibre pulp, but which is of such superior quality that it enables a superior paper to be produced solely from such short fibre material. When longer fibres are admixed with the short fibre pulp, in the manufacture of paper, a greatly reduced amount of long fibres can be used and these will not require any extended treatment in the beaters. The paper in this case will still be made up, for the most part, of the uniform short fibre pulp of superior character with the longer fibres admixed therewith.

It is one advantage of the present invention that it enables different woods to be cooked in admixture with each other and a satisfactory mixed pulp directly produced. In this case, the resulting pulp and the paper made therefrom will still be made of fibres of uniform character, since the fibres of the different woods, although differing from each other, will nevertheless be of substantially uniform character so far as the fibres of each wood are concerned.

As an example of the application of the invention to the treatment of mixed woods, we may mention the cooking of poplar wood (which may be admixed with a small amount of bass wood) with a regulated amount of spruce wood. The amount of spruce wood ordinarily will be small, say 5 to 10% or even less, although more can be used where an increased admixture of long fibre pulp is desired. In the cooking of such a mixture of woods, the procedure will be similar to that above described in connection with the treatment of poplar wood, although both the pulp and the residual liquors will be modified, due to the different character of

the admixed spruce fibres of the pulp and to the somewhat different character of the non-fibrous constituents produced from this spruce wood.

As another instance of the application of the invention to the treatment of mixed woods, we will mention the treatment of poplar wood with the addition or admixture of a small amount of other hard woods, and particularly of hard woods of considerably increased weight or density, such as birch, beech and maple, either separately or in combination. These heavy hard woods contain a greatly increased weight of both pulp fibres and non-fibrous material, so that for equal quantities of wood (by volume) the amount of pulp produced and also the amount of soluble constituents requiring removal in the residual liquors will be correspondingly increased. Where the admixtures of these dense hard woods is only to the extent of a few per cent, say up to 5 or 10%, this increased amount of both fibres and non-fibrous constituents will not require any great variation in the process, although the amounts of reagents used in the cooking liquor can be somewhat increased to take care of the increased amount of non-fibrous constituents to be dissolved away from the pulp fibres.

Where the amounts of dense hard woods used in admixture with poplar wood are increased to a greater extent, for example, to an amount similar to that of the poplar wood, the problem is presented of treating a charge which, in total weight of wood, may be half as much again as the weight of the ordinary charge of poplar wood in a digester of the same size. Where the dense hard woods, such as beech, birch and maple, etc., are treated by themselves, either separately or in admixture with one another, the total weight of the wood will be radically greater than the weight of poplar wood, normally chargeable into the same digester. The weight of the hard woods may be as much as twice that of the poplar wood, while the amounts of non-fibrous constituents which must be separated from the fibres may be even greater in proportion, because of the lesser content of fibres and the increased content of non-fibrous constituents which certain of the dense hard woods contain.

When the dense hard woods are cooked by themselves, the cooking liquor will require to be greatly increased in strength, in order that a digester full of the hard wood chips may be satisfactorily cooked, and it may advantageously be increased in amount, as compared with the amount used with poplar wood. It is an advantage of the present invention, however, that even these dense woods can be cooked, either by themselves or in admixture with varying amounts of poplar (and similar) wood. With these

6 dense woods, however, the same ratio of caustic soda to sodium sulphite need not ordinarily be used that would be used in the treatment of poplar wood. In general, the 5 increase in cooking reagents may be made up, for the most part, of sodium sulphite, so that in any case, the amount and strength of caustic soda in the composite cooking liquor is kept below the amount which will cause 10 any considerable injury to the fibres of the pulp produced. For example, with dense hard wood the cooking liquor may be made up of caustic soda and sodium sulphite in approximately equal amounts, so far as their 15 sodium content is concerned, and such a composite cooking liquor can be used of a strength somewhat less than double the strength of a cooking liquor which would be similarly used in the treatment of poplar 20 wood, and in somewhat increased amounts, although the amounts and strengths of the cooking liquor can be somewhat varied as well as the proportions of caustic soda and sodium sulphite which the cooking liquor 25 contains. In cooking heavy hardwoods it is desirable to increase the volume above the amount used with poplar wood.

In cooking mixtures of poplar wood and dense hard woods, where the poplar wood is 30 not the predominating wood, the strengths and amounts of the reagents in the cooking liquor can be regulated and controlled in accordance with the amounts of non-fibrous materials which the woods contain, while 35 maintaining the caustic soda of a strength and concentration which will avoid any considerable injury to the pulp fibres, and making up the balance of the cooking reagents mostly of sodium sulphite.

40 Even where different woods are cooked in admixture with each other, the present invention enables the different woods to be satisfactorily cooked without overcooking part of the wood while completing the cooking 45 of the rest, which may require a somewhat shorter time. By cooking mixed woods in this way, mixed pulps may be directly produced containing fibres of different characteristics produced from different woods. We have found that the fibres from different 50 woods possess different properties and characteristics which enable them to be distinguished from each other as well as from fibres produced, for example, from poplar wood by the ordinary soda process.

The residual liquors produced in the new process of the present invention can be readily treated for the regeneration of the cooking liquors by subjecting them to evaporation 55 in multiple effect evaporators and by calcining the resulting concentrated liquor in rotary calcining furnaces such as are used in the calcining of black liquor from the ordinary soda process. Owing to the decreased amount of wood substance contained

in solution in the residual liquors (from poplar wood), the liquors are less gummy in character and give less trouble in the evaporators from foaming or gumming, etc. The liquor, from the strong liquor tank, of a 70 strength of around 14 to 14.5° Twaddell at a temperature of 155 to 160° F. can be readily concentrated in quadruple effect evaporators to 60 or 65° Twaddell, or even higher, 75 at a temperature of 140 to 144° F. The concentrated liquor can then be fed to the rotary calcining furnaces such as are used in treating black liquors from the ordinary soda process.

We have found that, although the residual 80 liquors contain a considerable amount of combined sulphur they can nevertheless be calcined in the rotary furnaces without driving off the entire amount of the combined sulphur. We have also found that under 85 certain conditions sodium sulphite comes from the rotary calcining furnaces without any considerable amount of reduction by the admixed organic matter, a few per cent, only of sulphide being formed. The presence 90 of a few per cent of sodium sulfide is, however, advantageous in the cooking liquor, supplementing the action of the caustic soda and of the sodium sulfite. The rotary calcining furnaces may, for example, have a diameter of about 9 feet and a length of about 95 16 feet and may be heated by coal fire. The concentrated residual liquor from the multiple effect evaporators, concentrated to about 60-65° Twaddell can be fed into the 100 rotary furnaces at one end and the calcined product discharged at the other. With proper control of the calcination, such that fusion of the discharged product is avoided as 105 much as possible, the sulphite comes from the furnace in considerable amount.

The calcined product can then be leached, for example, by introducing it into water and agitating the water, or by otherwise carrying out the leaching operation. By countercurrent leaching a solution can be obtained up to 27-31° Twaddell. This liquor can be subjected to causticizing with lime to convert its contained sodium carbonate for the most part into caustic soda, using, for example, 53 or 54 parts of calcium oxide to 100 parts of sodium carbonate. The sulphite contained in the liquor is preferably not causticized, and the amount of lime should be kept sufficiently low to avoid this. The causticizing operation can be carried out by heating and agitating for a sufficient period of time to carry the causticizing to the desired degree. Some sodium carbonate will usually be left uncausticized in the resulting liquor, which will be made up for the most part of caustic soda, resulting from the causticizing operation, and sodium sulphite. Some small and incidental amount of sodium sulphide may also be present, produced dur- 130

ing the calcination, but we have found that, by avoiding smelting of the charge during calcination, there is no building up of sulphide to an objectionable degree nor is there 5 any excessive building up of sulphate, but the sulphite in considerable part passes through the furnace and is recovered for further use, while such small and incidental amounts of sodium sulphide as may be 10 formed and as may be present in the regenerated liquor, are without any objectionable effect in the process when carried out with the regenerated cooking liquor, although such amounts of sodium sulphide can be 15 readily removed, if desired. Such amounts of sodium sulfide as are incidentally produced during the regeneration will when present supplement the action of the caustic soda and sodium sulfite, giving a composite 20 cooking liquor containing caustic soda, sodium sulfite and sodium sulfide, with the caustic soda in preponderating amount.

In order to make up for losses of caustic soda and sodium sulphite, a suitable amount 25 of dry soda ash, for example, may be added to the liquor before causticizing, while the necessary amount of sodium sulphite can be readily produced, for example, by burning sulphur in a small sulphur burner and absorbing the sulphur dioxide in a solution of soda ash or a solution which contains the sodium carbonate leached from the calcined 30 product above described. A convenient method of supplying sodium sulphite in the required amount is to absorb the sulphur dioxide from a sulphur burner in an absorption tower through which a solution of sodium carbonate is circulated containing around 130 to 140 grams of soda ash per 35 liter, or a part of the leach-liquor can be similarly used. The freshly made sodium sulphite solution may be added to the remainder of the cooking liquor either in the digester or before it enters the digester. The 40 regenerated cooking liquor may be separately introduced into the digester and the newly made sulphite liquor separately added, for example, adding 394 cubic feet of regenerated cooking liquor of 16° Twaddell at 45 60° F. together with about 66 cubic feet of freshly made sodium sulphite liquor of proper strength, this referring especially to poplar wood. Some residual liquor from a previous operation may be substituted for an 50 equal volume of water so that the total volume added remains about 460 cubic feet for the particular digester specified.

The cooking liquors thus produced can be used in carrying out the cooking operation 55 hereinbefore described.

When dense hard woods (for example birch, beech, maple, etc.) which have a considerably greater weight than poplar wood, the amount of non-fibrous constituents which the woods contain and which

must be removed by the cooking operation will be radically greater than in the case of poplar wood, assuming that a digester full of the wood is treated in each case. Along with the greatly increased amount of pulp 70 which can be produced from a digester charge of the hard woods, there will be a similar increase, or even a greater increase, in the amount of non-fibrous constituents present in the residual liquors, particularly 75 where the hard woods have a considerably increased per cent of non-fibrous constituents as compared with poplar wood. The residual liquors will accordingly contain a greatly increased content both of organic 80 and of inorganic constituents, such as combined sodium organic compounds and sulpho-organic compounds, etc. These residual liquors, of such increased concentration, can be somewhat diluted by admixture with 85 wash waters, but dilution to an objectionable degree can be readily prevented and the treatment of the more concentrated liquors presents added advantage because of the decreased amount of water to be removed and 90 the radically increased concentration of the constituents which the liquor contains. The treatment of the liquor can, however, be carried out in a manner similar to that above described in connection with the treatment of 95 residual liquors from the cooking of poplar wood.

It will thus be seen that the present invention provides a regenerative process of pulp manufacture in which the cooking liquor is 100 of a composite character, containing essentially caustic soda and sodium sulphite, and in which the residual liquors can nevertheless be readily treated for the regeneration therefrom of the cooking liquor containing 105 essentially the same ingredients. The process, when thus carried out as a regenerative process, is of a cyclic character, with cooking of the wood chips with the composite cooking liquor, evaporation of the residual liquor and calcination of the concentrated liquor, with regulation of the calcining operation, so that the chemicals are recovered without excessive loss, and with leaching of the calcined material and causticizing of 110 the leached liquor with lime, using a regulated amount of lime such that the major portion of the sodium carbonate is causticized.

From one view point, the process of the 115 present invention has features of similarity with the ordinary soda process, particularly in that the cooking liquor contains caustic soda as one of its characteristic ingredients. From the ordinary soda process, however, the process of the present invention is distinguished in many important respects, hereinbefore referred to. The cooking liquor, although it contains caustic soda as one of its 120 essential constituents, nevertheless has a 125

sufficiently mild action upon the wood due to the reduced amount and concentration of sodium hydroxide so that the objections of the ordinary soda process are largely avoided; while the use of a composite cooking liquor enables important additional advantages to be obtained. The present process retains many of the advantages of both the soda process and the acid sulphite process, while avoiding the strongly acid character of the latter and the objectionable alkaline strength of the cooking liquor of the former. The residual liquor produced according to the present invention is also of distinctive and characteristic composition. It contains less dissolved fibrous material and consequently less organic matter. It can be more readily evaporated without difficulty; and it acts in a characteristic way when subjected to calcination, and when the calcining operation is regulated in the manner above described. From the calcined material the new cooking liquor can be produced by regulated causticizing operation, regulated and controlled in the manner above indicated.

The pulp produced according to the present invention also is of an improved character and has fibres which differ in their composition and properties from those produced by the ordinary soda process. The improved properties of the fibre distinguish it in its handling throughout the mill, in the manner above described, and this improvement is noticeable in general mill operations. The pulp has a characteristic feel, has increased strength and is characterized by great uniformity while it runs freely through the mill, and paper made therefrom is safer in its production, while the paper produced has the improved and distinguishing properties above described. The process of the present invention, accordingly, presents advantages throughout the entire mill operations of a pulp and paper mill as compared with a mill operating the soda process and employing admixed soda and sulphite pulp for the manufacture of paper. The present invention makes it possible to eliminate the admixture of long fibre sulphite pulp with soda pulp for the manufacture of the heavier weights of book paper, while the paper produced according to the present invention is itself of improved quality.

A mill designed and constructed for the carrying out of the soda pulp process e. g., with poplar wood, can be transformed into a mill for carrying out the improved process of the present invention for treating poplar wood with few changes. The same equipment can be used in substantially the same manner in which it is now used in carrying out the soda process; but the carrying out of the present process will nevertheless result in a radical improvement in the opera-

tion of the mill, not only in the yield of pulp produced from the same amount of wood, but also in the ease with which the mill can be operated and kept in balance, with successive parts of the mill operating on schedule and in the improved quality and character of the products produced, i. e., residual liquor, pulp and paper. The improvements in the operation of the mill, as compared with the operation of the same mill with the soda process, are sufficiently marked so that they are noticeable even to the workmen throughout the mill, so that the workmen can readily tell the difference in the pulp by its "feel" and by the manner in which it can be handled and by the product produced.

In transforming a mill operating according to the soda process, for example, with poplar wood, into a mill operating according to the present invention, the transition is readily made. For example, sodium sulphite can be gradually introduced into the cooking liquor of one of a group of digesters, or into several digesters of the group, and, with the regeneration and recovery of sodium sulphite from the residual liquors, and the addition of further amounts of sodium sulphite, the amount of sodium sulphite can be gradually built up to the desired extent, and thereafter maintained by the addition of such further amounts as may be necessary to make up for losses. As the amount of sodium sulphite builds up in this way, the improvement in the pulp and in the handling of the pulp through the mill becomes noticeable even before the amount of sodium sulphite is increased to that which may finally be used in the process. A few per cent only of added sodium sulphite, with corresponding reduction in the amount of caustic soda, has a noticeable effect in improving the process, while an amount of sodium sulphite corresponding to about 10 per cent of the caustic soda, and with a corresponding reduction in caustic soda, results in an improvement in operations so radical in character that those operating the process can immediately notice it throughout the mill operations, and so that the yield in pulp produced will be increased to a considerable extent. The improvement will be noticeable, for example, in the color of the unbleached pulp, which, instead of being a dark brown, will have a reddish or pinkish cast, as well as in the brightness of the pulp and the whiteness of the bleached pulp, it being necessary in some instances of paper manufacture to add coloring material in the production of ordinary white paper because of the unusual whiteness of the bleached pulp as compared with the standard product for which the pulp was to be used.

Where book and magazine paper mills

- using pulp produced by the soda process have heretofore been obliged to purchase or produce long fibre sulphite pulp (made by the acid sulphite process) at an increased 5 cost (as compared with the value of soda pulp) in order to admix the sulfite and soda pulps to give a paper of the necessary quality and strength, the present invention enables the purchase or production of sulphite 10 pulp to be eliminated, or reduced to a minimum, and enables an improved paper to be produced solely from short fibre woods, e. g. poplar, without any admixture whatever of long fibres therewith. Where mills now 15 operate both the soda and the acid sulphite processes in order to manufacture the two kinds of pulp for admixture with each other, the present invention enables the plant to be readily converted in part or in whole to 20 the improved process which makes unnecessary the manufacture of two different kinds of pulps for admixture and which enables the mill to operate with a wider variety of woods which cannot be readily treated according to the common methods. In fact, 25 the wider range of application of the present invention is an important and characteristic advantage, inasmuch as it greatly extends the range of available woods for the manufacture of satisfactory pulp, and makes unnecessary the treatment of the more expensive pulp woods which are decreasing in available amount and correspondingly increasing in cost. 30
- 35 The present invention accordingly presents many and varied advantages which are largely cumulative in character and which include a wider range of application and of materials treated as well as improvements in the method of treatment and throughout the method of treatment, and in the products which the process produces.
- We claim:
1. The method of manufacturing pulp from wood which comprises cooking the wood under pressure with a cooking liquor containing caustic soda and sodium sulphite as its primary reagents, the amount of the sulphite not exceeding that of the caustic 45 soda.
  2. The method of manufacturing pulp from wood which comprises cooking the wood under pressure with a cooking liquor containing a preponderating amount of caustic soda and a lesser amount of sodium sulphite. 50
  3. The method of manufacturing pulp from wood which comprises cooking the wood under pressure with a cooking liquor containing a preponderating amount of caustic soda and an amount of sodium sulphite equivalent to about 10 to 25% of the amount of caustic soda. 55
  4. The method of manufacturing pulp from wood which comprises cooking the 60
- wood under pressure with a cooking liquor containing a preponderating amount of caustic soda and a lesser amount of sodium sulphite, separating the residual liquor from the pulp, concentrating the residual liquor, 70 and calcining the concentrated liquor to carbonize organic matter, leaching the calcined material, and causticizing the resulting solution to give a composite solution containing caustic soda and sodium sulphite. 75
5. The method of manufacturing pulp from wood which comprises cooking the wood under pressure and at an elevated temperature, with a cooking liquor containing caustic soda, sodium sulfite and sodium sulfide, the caustic soda being present in preponderating amount. 80
6. The regenerative method of manufacturing pulp from wood which comprises cooking the wood under pressure with a cooking liquor containing a preponderating amount of caustic soda and a lesser amount of sodium sulfite, separating the residual liquor from the pulp, subjecting the residual liquor to concentrating and calcining operations, dissolving the soluble compounds, and treating the resulting solution for the production of further amounts of cooking liquor, said treatment including a causticizing treatment. 85
7. The regenerative method of manufacturing pulp from wood which comprises cooking the wood under pressure with a cooking liquor containing a preponderating amount of caustic soda and a lesser amount of sodium sulfite, separating the residual liquor from the pulp, subjecting the residual liquor to concentrating and calcining operations, dissolving the soluble compounds, and treating the resulting solution for the production of further amounts of cooking liquor, said treatment including a causticizing treatment and the formation of additional sodium sulfite. 90
8. The regenerative method of manufacturing pulp from wood which comprises cooking the wood under pressure with a cooking liquor containing a preponderating amount of caustic soda and a lesser amount of sodium sulfite, separating the residual liquor from the pulp, subjecting the residual liquor to concentrating and calcining operations, the calcination being regulated to give a calcined product containing sodium carbonate and sodium sulfite, dissolving the soluble compounds and incompletely causticizing the same to reproduce a solution containing caustic soda and sodium sulfite for further use in the cooking process. 100
9. The regenerative method of pulp manufacture which comprises cooking the wood under pressure with a cooking liquor containing a preponderating amount of caustic soda and lesser amounts of sodium sulfite and sodium sulfide, separating the residual 105

- liquor from the pulp, concentrating the residual liquor, calcining the concentrated liquor under conditions to form some sodium sulfide, dissolving the soluble compounds, and treating the same to form further amounts of cooking liquor, said treatment including a causticizing treatment, and the formation of additional amounts of sodium sulfite.
10. The method of manufacturing wood pulp from wood which comprises cooking the wood under pressure with a cooking liquor containing caustic soda and sodium sulfite as primary reagents, the cooking liquor containing a preponderating amount of caustic soda and a lesser amount of sodium sulfite, and the cooking operation being carried out under a steam pressure of around 110 to 120 pounds.
11. The method of manufacturing pulp from wood which comprises cooking the wood under pressure and at an elevated temperature with a cooking liquor containing caustic soda in preponderating amount and also containing sodium sulfite in such amount that it represents from 10 to substantially 25% the total sodium present.
12. The method of manufacturing pulp from wood which comprises cooking the wood under pressure and at an elevated temperature with a cooking liquor containing about 50 to 60 grams per liter of caustic soda and about 10 to 25 grams per liter of normal sodium sulfite.
13. The method of manufacturing pulp from wood which comprises subjecting the wood to a cooking operation under pressure at an elevated temperature with a cooking liquor containing a preponderating amount of caustic soda, together with a smaller amount of sodium sulfite, and also containing sodium carbonate, the cooking operation being carried out with relief of gases from the top of the digester from time to time during the cooking operation.
14. As a new product, a pulp resulting from the cooking of wood with a composite cooking liquor containing a preponderating amount of caustic soda and a lesser amount of sodium sulphite, said pulp containing fibres of great uniformity and being free flowing.
15. As a new product, a pulp resulting from the cooking of short fibre wood with a composite cooking liquor containing a preponderating amount of caustic soda and a lesser amount of sodium sulphite, said pulp containing fibres of sufficient strength to permit the manufacture of paper therefrom without the admixture of long fibre pulp.
16. As a new product, a pulp resulting from the cooking of poplar wood with a cooking liquor containing a preponderating amount of caustic soda and a lesser amount of sodium sulphite, said pulp containing fibres of radically increased strength as compared with fibres resulting from the cooking of poplar wood by the ordinary soda process, and said pulp permitting the manufacture of superior paper therefrom without the admixture of long fibre pulp therewith.
17. As a new product, a paper made entirely of short fibre pulp resulting from the cooking of short-fibre wood with a composite cooking liquor containing a preponderating amount of caustic soda and a lesser amount of sodium sulphite.
18. As a new product, a paper made up entirely of poplar pulp (which may contain a small admixture of bass wood pulp) produced with a cooking liquor containing a preponderating amount of caustic soda and a lesser amount of sodium sulphite.
19. A residual liquor resulting from the cooking of wood with a composite cooking liquor containing a preponderating amount of caustic soda and a lesser amount of sodium sulphite.
20. As a new product, a paper made entirely of short fiber pulp, the short fiber pulp resulting from the cooking of short fiber wood with a cooking liquor containing a preponderating amount of caustic soda and a lesser amount of sodium sulfite.
21. As a new product, a paper comprising short fiber pulp resulting from the cooking of short-fiber wood with a composite cooking liquor containing a preponderating amount of caustic soda and a lesser amount of sodium sulphite.
22. As a new product, a paper comprising paper pulp containing fibers of substantially uniform length and properties produced by cooking the wood with a cooking liquor containing a preponderating amount of caustic soda and a lesser amount of sodium sulfite.
23. As a new product, a paper made from short fiber pulp admixed with a small amount of long fiber pulp, the short fiber pulp resulting from the cooking of short fiber wood with a cooking liquor containing a preponderating amount of caustic soda and a lesser amount of sodium sulfite.
24. The method of manufacturing pulp from wood which comprises cooking the wood under pressure and at an elevated temperature with a cooking liquor containing soda combined as sodium hydroxide and a lesser amount of soda combined as sodium sulfite and also including an amount of sodium sulfid which is less than the amount of sodium sulfite.
25. The method of manufacturing pulp from wood which comprises treating wood by means of a liquor containing soda as sodium hydroxide and lesser amounts of soda combined as sodium sulfite and as sodium sulfid, the amount of sodium sulfite being at least about ten percent (10%) of the amount of sodium hydroxide.

26. The method of manufacturing pulp which comprises treating cellulose-fibre-bearing material, including lignified material, by means of liquor containing soda combined as sodium hydroxide and lesser amounts of soda combined as sodium sulfite and as sodium sulfid, the amount of sodium sulfite being at least about ten percent (10%) of the amount of sodium hydroxide, and the amount of sodium sulfid being less than the amount of the sodium sulfite.

27. In a process for producing pulp from wood, the steps which include subjecting wood to a digesting treatment by means of liquor supplied with soda combined as sodium hydroxide and as sodium sulfite, the amount of sodium sulfite being at least about ten percent (10%) of the amount of the sodium hydroxide, and containing digestive material, exclusive of the sodium sulfite, alkaline to phenolphthalein, in an amount which is capable of digesting at least one-half of the non-fibrous organic content of the wood, and the digestion treatment being conducted so that fibres of the resulting material are readily separable from each other by mechanical treatment.

28. In a process for producing pulp from wood, the steps which include subjecting wood to a digesting treatment by means of liquor supplied with soda combined as sodium hydroxide and as sodium sulfite, the amount of sodium sulfite being at least about ten percent (10%) of the amount of the sodium hydroxide, and containing digestive material, exclusive of the sodium sulfite, alkaline to phenolphthalein, in an amount which is capable of digesting at least one-half of the non-fibrous organic content of the wood, and the digesting treating being conducted so as to separate from the fibres substantially all non-fibrous organic constituents without unduly weakening or injuring the resulting fibres.

45. 29. In a process for producing pulp from wood, the steps which include subjecting wood to a digesting treatment by means of liquor supplied with soda combined as sodium hydroxide and lesser amounts of soda combined as sodium sulfite and sodium sulfid, the amount of sodium sulfite being at least about ten percent (10%) of the amount of sodium hydroxide, and the amount of sodium hydroxide being less than would be required to digest a similar amount of the non-fibrous organic content of the wood if sodium hydroxide were the only reagent employed.

60. 30. In a process for producing pulp from wood, the steps which include subjecting wood to a digesting treatment by means of liquor supplied with soda combined as so-

dium hydroxide and as sodium sulfite, the amount of sodium sulfite being at least about ten percent (10%) of the amount of the sodium hydroxide, and the hydroxide being supplied in an amount which is capable of digesting at least one-half of the non-fibrous organic content of the wood.

31. In a process for producing pulp from wood, the steps which include subjecting wood to a digesting treatment by means of liquor supplied with soda combined as sodium hydroxide and as sodium sulfite, the amount of sodium sulfite being at least about ten percent (10%) of the amount of the sodium hydroxide, and the hydroxide being supplied in an amount which is capable of digesting at least one-half of the non-fibrous organic content of the wood, and the digesting treatment being conducted so that fibres of the resulting material are readily separable from each other by mechanical treatment, and the separated fibres are relatively strong as compared with chemical pulp from the same kind and quality of wood as produced by the conventional soda process.

32. In a process for producing pulp, the steps which include subjecting cellulose-bearing material, including ligneous material, to a digestion treatment by means of liquor supplied with alkali combined as alkali hydroxide, as alkali sulfite and as alkali sulfid, the amount of the alkali sulfite being at least as large as the amount of the alkali sulfid, and the hydroxide being supplied in an amount which is capable of digesting at least one-half of the non-fibrous organic content of the cellulose-bearing material.

33. In a process for producing pulp from wood, the steps which include subjecting wood to a digestion treatment by means of liquor supplied with soda combined as sodium hydroxide, as sodium sulfite and as sodium sulfid, the amount of the sodium sulfite being at least as large as the amount of the sodium sulfid, and the hydroxide being supplied in an amount which is capable of digesting at least one-half of the non-fibrous organic content of the wood, and the digestion treatment being conducted so as to render fibres of the resulting material readily separable from each other by mechanical treatment, and the resulting fibres being sufficiently free from non-fibrous organic material and of sufficient strength to be employed in the formation of the fibrous structure of machine-made paper weighing between 30 and 70 pounds per ream of 500 sheets, each 25 inches by 38 inches.

In testimony whereof we affix our signatures.

LINN BRADLEY.  
EDWARD P. MCKEEFE.